

## UNITED STATES PATENT OFFICE

1,976,881

UNHAIRING BATH AND PROCESS FOR  
TREATING HIDESNorman D. Harvey, Jr., Providence, R. I., assignor  
to Carbide and Carbon Chemicals Corporation,  
a corporation of New YorkNo Drawing. Application March 15, 1932,  
Serial No. 599,059

20 Claims. (Cl. 149—2)

The invention relates to baths for unhauling hides, and includes a process for treating hides to effect the removal of hair therefrom. Unhauling baths are useful in recovering wool or other hair for textile purposes, but their principal application is in the preparation of hides for tanning.

Hides are normally received at the tannery after curing by sun-drying or salting. At the 10 tannery the hides are soaked to cleanse and rehydrate them. Soaking is usually done in plain water and is continued until all the salt, in the case of salt cured hides, is eliminated from the hide. The hides are thereafter unhaired, 15 plumped, and finally tanned.

In general practice the unhauling and plumping operations are carried out together, as by 20 treating the hides for two or three days in a bath prepared by suspending lime in water, and then adding sodium sulfide. Such a bath decomposes the epidermis, or outer layer of the hide; and since the epidermis lines the hair follicles and 25 grips the hairs the latter are loosened so that they can be removed mechanically. At the same time the corium (which underlies the epidermis and forms the substance of the finished leather) swells, takes on a firmer texture, and is otherwise modified so that it becomes amenable to 30 tanning. This effect is called plumping, and additional agents may or may not be added to the bath to produce the desired degree of plumping.

In accordance with the invention, aliphatic primary, secondary, or tertiary amines in physical or chemical combination with sulfur are used as 35 dehauling agents. Thus, amine sulfides or sulfites, sulfur dissolved in amine solutions, and finely dispersed or colloidal sulfur in conjunction with known depilatory agents, alone or in conjunction with lime are examples of my improved 40 dehauling agents.

The invention is illustrated by the following examples, but is not to be considered as limited thereby:

I. Hydrogen sulfide gas was bubbled through a 45 50% solution of ethylene diamine in water. Heat was evolved and a yellow solution was obtained. This product will be designated as ethylene diamine sulfide.

An unhauling bath was prepared equal to four 50 times the weight of soaked calfskin to be unhaired. This bath contained 1% of the weight of soaked hides of ethylene diamine sulfide, and 10% of the weight of soaked hides of a 20% suspension of freshly slaked lime. After 24 hours of treatment in this solution the calfskins were

readily unhaired. The same amount of lime alone did not unhaire in several days time.

Ethylene diamine sulfide was as effective as the same quantity of sodium sulfide (a common depilatory agent). In each case the hair was destroyed, but the hides after the ethylene diamine sulfide treatment were softer and lighter in color than those unhaired with sodium sulfide. Ethylene diamine also is advantageous in that it serves as a carrier for sulfides, and retains as a suspension in the solution any calcium sulfide which may be formed. Calcium sulfide as such is insoluble and is valueless in unhauling.

Other amines, including methylamine and mono, di, and triethanolamines may be used in 70 the same manner as ethylene diamine, and their sulfides are satisfactory unhauling agents.

II. Flowers of sulfur were dissolved in 50% 75 solutions of triethanolamine, monoethanolamine, and ethylene diamine; in a 34% solution of methylamine; and in a 95% solution of diethanolamine. Ethylene diamine dissolved the most sulfur, methylamine about the same amount, mono and diethanolamine a lesser amount, and triethanolamine the least.

A crystalline flaky precipitate which was quite 80 stable was obtained from the ethylene diamine solution. Calfskins were satisfactorily unhaired after 70 hours treatment in a solution containing 5% of this precipitate and 5% of lime based 85 on the weight of soaked skins. All of the amine solutions containing dissolved sulfur exhibited increased unhauling power over ordinary depilatory or plain amine solutions. In each case the time required for satisfactory unhauling was decreased by increasing the amount of amine-sulfur 90 solution in the unhauling bath. It was also discovered that a mixture of equal parts of the ethylene diamine and methylamine sulfur solutions in conjunction with lime was better than 95 either solution alone.

The solutions described in this example are 100 true solutions rather than chemical combinations, since an excess of water will precipitate the sulfur. The amine-sulfur solutions possess the advantage of producing lighter colored and softer hides than known depilatories, and unlike strongly alkaline depilatories, such as sodium sulfide, they do not destroy the hair.

III. Solutions of amine sulfites were prepared by bubbling sulfur dioxide into the amine solutions. These solutions were then used as in Example I, and the following amine sulfites were found to be satisfactory depilatories: ethylene di- 110

amine, methylamine, monoethanolamine, and diethanolamine.

IV. The amine sulfides described in Example I may be made into pastes for unhauling sheepskins. Of these, ethylene diamine, methylamine, and monoethanolamine sulfides produced the best results. For example, a paste consisting of 5% ethylene diamine sulfide, 15% lime and 80% water unhaired satisfactorily in 20 to 24 hours. The paste is applied to the flesh side of the skin in order to avoid destroying the wool.

The advantages of amine sulfides in depilatory pastes for sheepskins may be listed as follows, in which the new unhauling agents are compared

15 to sodium sulfide, the usual depilatory:

Sodium sulfide is a solid, difficult to dissolve, and its solutions and pastes must be kept hot to prevent crystallization of the sodium sulfide. The sodium sulfide crystallizes in the brushes by 20 which the paste is applied and quickly destroys them.

Amine sulfides may be handled in concentrated solutions, and when solid are readily dissolved. The amine sulfides are soluble in cold water, and 25 the pastes may be used cold. The amine sulfide does not crystallize out of the paste easily. Amine sulfide pastes are thicker in consistency than those made from sodium sulfide. Thin pastes tend to flow over the edges of sheep skins, 30 and destroy the wool.

In all cases, hides unhaired with amine-sulfur chemical or physical combinations are in better condition than those unhaired with previously known agents. The hair is completely removed without leaving the roots in the skin. The amine 35 unhauling baths exert a distinct cleansing effect on the hides producing a cleaner, lighter colored hide. The hide also has a softer, finer texture when treated in accordance with the invention. In those cases in which the hair is not destroyed 40 the hair removed is in better condition since all of the fiber length, including the roots of the hairs is recovered.

In addition to the unhauling baths disclosed, 45 modified embodiments of the invention are possible. For example, alkali hydroxides, such as sodium or potassium hydroxide, or other strong alkalies in small amounts may be added to the unhauling baths of my invention. Also, I have 50 found that finely dispersed or colloidal sulfur alone in conjunction with lime in unhauling baths increases the efficaciousness of such baths.

I claim:

1. An unhauling bath containing sulfur in physical combination with a depilatory agent comprising an aliphatic amine.

2. An unhauling bath containing sulfur in physical combination with depilatory agents comprising aliphatic amines and an inorganic compound 60 having an alkaline reaction.

3. An unhauling bath containing sulfur in physical combination with depilatory agents comprising an aliphatic amine and lime.

4. An unhauling bath containing depilatory 65 agents of the group consisting of chemical and physical combinations of sulfur with aliphatic amines.

5. An unhauling bath containing depilatory agents of the group consisting of chemical and physical combinations of sulfur with aliphatic amines in conjunction with inorganic compounds 70 having an alkaline reaction.

6. An unhauling bath containing depilatory agents of the group consisting of chemical and physical combinations of sulfur with aliphatic amines in conjunction with lime.

7. An unhauling bath containing depilatory 80 agents of the group comprising the sulfites of aliphatic amines.

8. An unhauling bath containing depilatory agents of the group comprising the sulfites of ethylene diamines, methylamine, monoethanolamine, diethanolamine, and triethanolamine. 85

9. An unhauling bath containing depilatory agents of the group comprising the sulfites of aliphatic amines in conjunction with lime.

10. An unhauling bath containing depilatory 90 agents of the group comprising the sulfites of ethylene diamine, methylamine, monoethanolamine, diethanolamine, and triethanolamine in conjunction with lime.

11. An unhauling bath containing depilatory 95 agents of the group consisting of physical solutions of sulfur in solutions of aliphatic amines.

12. An unhauling bath containing depilatory agents of the group consisting of physical solutions of sulfur in solutions of ethylene diamine, 100 methylamine, monoethanolamine, diethanolamine, and triethanolamine.

13. An unhauling bath containing depilatory agents of the group consisting of physical solutions of sulfur in solutions of ethylene diamine, 105 methylamine, monoethanolamine, diethanolamine, and triethanolamine in conjunction with lime.

14. Process of unhauling hides which comprises subjecting the hides to the action of an unhauling 110 bath containing sulfur in physical combination with a depilatory agent comprising an aliphatic amine until the hair is loosened.

15. Process of unhauling hides which comprises subjecting the hides to the action of an unhauling 115 bath containing sulfur in physical combination with depilatory agents comprising aliphatic amines and lime until the hair is loosened.

16. Process of unhauling hides which comprises subjecting the hides to the action of an unhauling 120 bath containing depilatory agents of the group consisting of chemical and physical combinations of sulfur with aliphatic amines until the hair is loosened.

17. Process of unhauling hides which comprises subjecting the hides to the action of an unhauling 125 bath containing depilatory agents of the group consisting of chemical and physical combinations of sulfur with aliphatic amines in conjunction with lime until the hair is loosened.

18. Process of unhauling hides which comprises 130 subjecting the hides to the action of an unhauling bath containing depilatory agents of the group comprising the sulfites of aliphatic amines until the hair is loosened.

19. Process of unhauling hides which comprises 135 subjecting the hides to the action of an unhauling bath containing depilatory agents of the group consisting of physical solutions of sulfur in solutions of aliphatic amines.

20. Process of unhauling sheepskins which comprises applying to the flesh side of the sheepskins 140 a paste containing a sulfide of an aliphatic amine of the group comprising ethylene diamine, methyl amine, and monoethanolamine and lime, and allowing said paste to remain on said skin until the 145 wool is loosened.

NORMAN D. HARVEY, JR.